

## [54] DEVELOPER COMPOSITION FOR ELECTROPHOTOGRAPHY

[75] Inventors: Eizi Morimoto; Kuniyasu Kawabe; Tetuhiro Semura, all of Wakayama, Japan

[73] Assignee: KAO Corporation, Tokyo, Japan

[21] Appl. No.: 814,628

[22] Filed: Dec. 30, 1991

## [30] Foreign Application Priority Data

Jan. 18, 1991 [JP] Japan ..... 3-4414

[51] Int. Cl.<sup>5</sup> ..... G03G 9/087

[52] U.S. Cl. ..... 430/106.6; 430/109

[58] Field of Search ..... 430/106.6, 109, 110, 430/111

## [56] References Cited

## U.S. PATENT DOCUMENTS

2,297,691 10/1942 Carlson ..... 430/56  
 4,863,824 9/1989 Uchida et al. ..... 430/109  
 4,940,644 7/1990 Matsubara et al. ..... 430/109  
 5,037,715 8/1991 Hagiwara et al. ..... 430/109

## FOREIGN PATENT DOCUMENTS

3808448 9/1988 Fed. Rep. of Germany ..  
 60-214368 10/1935 Japan ..  
 4223910 11/1942 Japan ..  
 4324748 10/1943 Japan ..  
 57-109825 7/1982 Japan ..  
 57-208559 12/1982 Japan ..  
 58-11954 1/1983 Japan ..  
 59-7960 1/1984 Japan ..  
 59-9669 1/1984 Japan ..

59-11902 1/1984 Japan ..  
 59-29255 2/1984 Japan ..  
 59-29256 2/1984 Japan ..  
 59-29257 2/1984 Japan ..  
 59-29258 2/1984 Japan ..  
 59-228861 12/1984 Japan ..  
 60-4947 1/1985 Japan ..

## OTHER PUBLICATIONS

Electrophotography: The Society Journal, vol. 22, No. 1, 1983, pp. 7-16.

Electrophotography: The Society Journal, vol. 25, No. 1, 1986, pp. 52-58.

Primary Examiner—John Goodrow

Attorney, Agent, or Firm—Birch, Stewart, Kolasch & Birch

[57]

## ABSTRACT

A developer composition for electrophotography comprising a binding resin and a colorant, said binding resin comprising a first linear polyester having a softening point, T<sub>sp</sub>, in the range of from 105° C. to 170° C. exclusive, and a second linear polyester having a softening point, T<sub>sp</sub>, in the range of from 80° C. to 105° C. exclusive and lower than that of the first linear polyester by at least 10° C., the weight ratio of the first linear polyester to the second linear polyester being (80:20) to (20:80) is disclosed.

The developer composition of the present invention is excellent in the hot offset resistance, low temperature fixation, smoothness of fixed face, blocking resistance and transparency.

8 Claims, No Drawings

DEVELOPER COMPOSITION FOR  
ELECTROPHOTOGRAPHY

## FIELD OF THE INVENTION

The present invention relates to a developer composition for electrophotography suitable for use in a color developer of a full color copying machine for developing an electrostatic charge image in electrophotograph, electrostatic recording, electrostatic printing, etc.

## DESCRIPTION OF THE RELATED ART

In electrophotography, many processes are known as described in U.S. Pat. No. 2,297,691 and Japanese Patent Publication Nos. 23910/1967 and 24748/1968. Among them, a general process comprises forming an electrical latent image on a photoreceptor by various means through the utilization of a photoconductive substance, developing the latent image with a toner, optionally transferring the resultant toner image to a transfer material, such as paper, and fixing the image by heat, pressure or solvent vapor to obtain a duplicate.

Various processes and apparatus have been developed regarding the above-described final step, i.e., the step of fixing a toner image on a sheet, such as paper. The process most commonly used in the art at the present time is a press bonding heating system.

In the press bonding heating system in which a heating roller is used, the fixation is conducted by passing a fixing sheet through a heating roller having a surface comprising a material which is releasable from a toner in such a manner that the toner image on the fixing sheet is brought into contact with the surface of the heating roller under pressure. In this process, since the surface of the heating roller is brought into contact with the toner image under pressure, the heat efficiency in the case where the toner image is fused to the fixing sheet is so good that the fixation can be rapidly conducted, which renders this process very useful in high-speed electrophotographic equipment. In the above-described process, however, since the surface of the heating roller comes into contact with the toner image in a molten state under pressure, part of the toner image adheres to and is transferred onto the surface of the fixing roller and re-transferred onto the next fixing sheet, so that there occurs the so-called "offset" phenomenon, which may stain the fixing sheet. The avoidance toner adhering onto the surface of the heat fixing roller is viewed as one requirement for the heat roller fixation system.

In other words, the development of a binder resin for a toner having a broad fixation temperature region and a higher offset resistance has been described in the art.

Two-color copying machines, and full color copying machines as well, have been studied, and many of them have been put to practical use. For example, there are reports on the color reproducibility and tone reproducibility in "Journal of the Society of the Electrophotography of Japan", vol. 22, No. 1 Page 7 (1983) and "Journal of the Society of the Electrophotography of Japan", vol. 25, No. 1, p. 52 (1986).

As opposed to television images, photographs and color prints, the full color electrophotographic image is not immediately compared with the original, and full color electrophotographic images, which have been put to practical use, are not always satisfactory for persons who get used to seeing a color image processed more beautifully than the original.

In full color electrophotography wherein development is conducted a plurality of times, and it is necessary to put several kinds of toner layers different from each other in color on an identical substrate, color toners used in such electrophotography should satisfy the following requirements.

- (1) In order to avoid the inhibition of color reproducibility derived from the irregular reflection of light, the fixed toner should be placed in a substantially molten state such that the form of the toner particles cannot be distinguished.
- (2) The color toner should be transparent to such an extent that the color reproducibility of the underlying layer having a different color toner is not inhibited.

Thus, the toner for a full color copying machine is required to not only have a broad fixation temperature region but also have transparency and flatness in the fixed face.

In order to broaden the fixation temperature region of the polyester, Japanese Patent Laid-Open Nos. 208559/1982, 11954/1983 and 228861/1984 each disclose a method in which an offset preventive agent is used. In these methods, however, the fluidity lowers, the toner impaction to the carrier is accelerated in a binary system, and the transparency is lost in the case of a full color toner. Japanese Patent Laid-Open Nos. 109825/1982 and 11902/1984 each discloses a method of improving the offset resistance through the use of a polycarboxylic acid to form a three-dimensional structure in the polyester. In these methods, although the offset resistance can be improved, when a large proportion is occupied by a high molecular region, the elasticity becomes very large when a toner is prepared therefrom, so that the fixed face does not become flat when the fixation is conducted at relative low temperature. This brings about a problem of color reproducibility when it is used in a full color toner. Further, Japanese Patent Laid-Open Nos. 7960/1984, 9669/1984 and 29255-29258/1984 each discloses a method of forming a three-dimensional structure in the polyester through the use of a tricarboxylic or higher polycarboxylic acid or a triol or a higher polyol. In the methods described in Japanese Patent Laid-Open Nos. 29255 and 29256/1984, however, the fixation is poor due to the absence of a soft segment, such as a succinic acid derivative. Further, in the methods described in Japanese Patent Laid-Open Nos. 7960/1984, 9669/1984, 29257/1984 and 29258/1984, since succinic acid substituted with an alkyl group is used, the toner exhibits fixation superior to that of the toners disclosed in Japanese Patent Laid-Open Nos. 29255 and 29256/1984 but is still unsatisfactory in fixation when it is used in a full color toner.

As described above, it is very difficult to simultaneously satisfy the broadening of the fixation temperature region and the toner properties, i.e., charging properties, fluidity, durability, transparency and smoothness of the fixed face.

## SUMMARY OF THE INVENTION

An object of the present invention is to provide a novel developer composition for electrophotography which eliminated the above-described problems.

Another object of the present invention is to provide a developer composition for electrophotography comprising a toner for heat roller fixation capable of forming a smooth fixed face for the purpose of avoiding the

inhibition of color reproduction derived from irregular reflection.

A further object of the present invention is to provide a developer composition for electrophotography comprising a toner for heat roller fixation which has excellent fluidity, no agglomeration and has excellent impact resistance.

Further scope of the applicability of the present invention will become apparent from the detailed description given hereinafter. However, it should be understood that the detailed description and specific examples, while indicating preferred embodiments of the invention, are given by way of illustration only, since various changes and modifications within the spirit and scope of the invention will become apparent to those skilled in the art from this detailed description.

The present inventors have made intensive studies with a view toward attaining the above-described objects and, as a result, have completed the present invention.

Specifically, the present invention relates to a developer composition for electrophotography comprising a binding resin and a colorant, said binding resin comprising a first linear polyester having a softening point,  $T_{sp}$ , in the range of from 105° C. to 170° C. exclusive, and a second linear polyester having a softening point,  $T_{sp}$ , in the range of from 80° C. to 105° C. exclusive and lower than that of the first linear polyester by at least 10° C., the weight ratio of the first linear polyester to the second linear polyester being (80:20) to (20:80).

It is preferable that the first linear polyester and the second linear polyester each comprises an acid component originated from an aliphatic dicarboxylic acid and/or acid anhydride thereof in an amount of 50% or more by mole, based on the entire acid component.

It is preferable that the first linear polyester and the second linear polyester each comprises an alcohol component originated from a compound represented by the following general formula (1) as a main component of its alcohol component.



wherein R stands for an ethylene group or a propylene group and x and y are each an integer, provided that the average value of the sum of x and y values is 2 to 7.

Furthermore, it is preferable that the glass transition temperature of the first linear polyester and the second linear polyester each is 40° to 80° C.

The binding resin is preferably comprised °F. 70 to 100% by weight of the total amount of the first linear polyester and the second linear polyester, based on the entire binding resin.

The binding resin comprises more preferably 70 to 100% by weight of the total amount of the first linear polyester and the second linear polyester and 30 to 0% by weight of styrene-acrylic resin, based on the entire binding resin.

The developer composition of the present invention, preferably further comprises a low molecular weight polyolefin and/or a magnetic impalpable powder.

## DETAILED DESCRIPTION OF THE INVENTION

The constitution of the present invention will now be described in detail. In the above-described first polyester, when the softening point,  $T_{sp}$ , is higher than the above-described range, the low-temperature fixation, the smoothness of the fixed face, the transparency and grindability become lower, while when the softening point,  $T_{sp}$ , is lower than the above-described range, the hot offset resistance and the blocking resistance become lower.

In the above-described second polyester, when the softening point,  $T_{sp}$ , is higher than the above-described range, the low-temperature fixation, the smoothness of the fixed face, the transparency and grindability become lower, while when the softening point,  $T_{sp}$ , is lower than the above-described range, the hot offset resistance and the blocking resistance become lower.

Basically, when the difference in the softening point,  $T_{sp}$ , between the above-described first polyester and the above-described second polyester contained in the developer composition of the present invention is 10° C. and more, the excellent properties of the individual polyesters are exhibited. On the other hand, when the difference in the softening point,  $T_{sp}$ , is less than 10° C., the expression of excellent properties of each of the first polyester and the second polyester are suppressed, such that some of the properties among those of hot offset resistance, low temperature fixation, transparency, smoothness of the fixed face and blocking resistance are adversely affected.

The blending weight ratio of the above-described first polyester to the above-described second polyester is (80:20) to (20:80), particularly preferably (70:30) to (30:70). When the blending weight ratio of the above-described first polyester is higher than the above-described range, the low temperature fixation and the smoothness of the fixed face are liable to be reduced. On the other hand, when the blending weight ratio of the first polyester is lower than the above-described range, the hot offset resistance and the blocking resistance are liable to be reduced.

Each of the above-described first polyester and the second polyester contains an acid component originated from an aliphatic dicarboxylic acid monomer which forms a relatively soft segment, preferably in an amount of 50% by mole or more based on the entire acid component. In this case, the low temperature fixation, the smoothness of the fixed face and the transparency become better.

It is preferred that the first polyester and the second polyester each further comprises an alcohol component originated from a diol represented by the following general formula (1) as a main alcohol component.



wherein R stands for an ethylene group or a propylene group and x and y are each an integer, provided that the average value of the sum of x and y values is 2 to 7.

The presence of the above-described alcohol component (the alcohol component originated from a diol represented by the general formula (1)) as the constitu-

ent unit contributes to a further improvement in the hot offset resistance, low temperature fixation and blocking resistance of the toner.

The glass transition point,  $T_g$ , of the first polyester and the second polyester each is preferably 40° to 80° C. A further improvement in the hot offset resistance, low temperature fixation and blocking resistance can be attained through the selection of the polyesters having a glass transition point falling within the above-described range. Specifically, when the glass transition point,  $T_g$ , is higher than the above-described range, the low temperature fixation and the smoothness of the fixed face are liable to be lower. On the other hand, when the glass transition point,  $T_g$ , is lower than the above-described range, the blocking resistance is liable to be lower.

In the present invention, the monomers used for the synthesis of the first polyester and the second polyester are basically the following dihydroxy alcohol or diol monomers and dicarboxylic acid monomers.

Examples of the dihydroxy alcohol monomer include etherified bisphenol, ethylene glycol, diethylene glycol, triethylene glycol, 1,2-propylene glycol, 1,3-propylene glycol, 1,4-butanediol, neopentyl glycol, 1,4-butenediol, 1,5-pentanediol, 1,6-hexanediol, 1,4-cyclohexanediethanol, dipropylene glycol, polyethylene glycol, polypropylene glycol, polytetramethylene glycol, bisphenol A and hydrogenated bisphenol A.

Among them, etherified bisphenol is particularly effective. Specific examples thereof include polyoxypropylene (2.2)-2,2-bis(4-hydroxyphenyl)propane, polyoxypropylene(3.3)-2,2-bis(4-hydroxyphenyl)propane, polyoxyethylene(2.0)-2,2-bis(4-hydroxyphenyl)propane, polyoxypropylene (2.0)-polyoxyethylene(2.0)-2,2-bis(4-hydroxyphenyl)propane and polyoxypropylene(6)-2,2-bis(4-hydroxyphenyl)propane.

Preferred examples of the dicarboxylic acid monomer include aliphatic dicarboxylic acids such as maleic acid, fumaric acid, citraconic acid, itaconic acid, glutaconic acid, succinic acid, adipic acid, sebacic acid, azelaic acid, malonic acid, n-dodecylsuccinic acid, isododecylsuccinic acid, n-dodecylsuccinic acid, isododecylsuccinic acid, n-octenylsuccinic acid, n-octylsuccinic acid and anhydrides or lower alkyl esters of these acids. If necessary, it is also possible to use aromatic dicarboxylic acids such as phthalic acid, isophthalic acid, terephthalic acid and anhydrides or lower alkyl esters of the above-described acids.

In the present invention, the softening point,  $T_{sp}$ , and the glass transition point,  $T_g$ , are defined respectively as values measured by the following methods.

#### Softening Point, $T_{sp}$

The softening point is defined as a temperature corresponding to  $\frac{1}{2}$  of the height from the flow initiation point to the flow termination point in the case where a sample having an area of 1 cm<sup>2</sup> is melt-flowed under conditions of a die pore diameter of 1 mm, a pressure of 20 kg/cm<sup>2</sup> and a temperature rise rate of 6° C./min through the use of a Koka flow tester "CFT-500" (manufactured by Shimadzu Corporation).

#### Glass Transition Point, $T_g$

A sample is heated to 100° C. by means of a differential scanning calorimeter (manufactured by Seiko Instruments Inc.), maintained at that temperature for 3 min and then cooled to room temperature at a temperature reducing rate of 10° C./min. In this sample, the measurement is conducted at a temperature increase of

10° C./min to obtain a curve. The intersection of a line extending from the base line of the curve at a portion below the glass transition temperature and a tangential line having the maximum gradient between the rising portion of the peak and the vertex of the peak is determined, and the temperature at that intersection is defined as the glass transition temperature,  $T_g$ .

The developer composition of the present invention contains the above-described first polyester and the above-described second polyester as indispensable components. The first polyester and the second polyester may be previously melt-blended with each other. The developer composition further contains a colorant, and, if necessary, may contain the other additives and resins besides first and second polyesters.

Low molecular weight polyolefins can be preferably used as the other additives. Specifically, low molecular weight polyethylene and polypropylene, etc. may be preferably used, and the softening point thereof as determined by the ring-and ball method is preferably 70° to 150° C., further advantageously 120° to 150° C. The incorporation of the above-described low molecular weight polyolefin contributes to further improvement in the hot offset resistance.

Examples of the above-described colorant include carbon black, nigrosine dyes (C. I. No. 50415B), aniline blue (C. I. No. 50405), chalco oil blue (C. I. azoic Blue 3), chrome yellow (C. I. No. 14090), ultramarine blue (C. I. No. 77103), de Pont oil red (C. I. No. 26105), quinoline yellow (C. I. No. 47005), methylene blue chloride (C. I. No. 52015), phthalocyanine blue (C. I. No. 74160), malachite green oxalate (C. I. No. 42000), lamp black (C. I. No. 77266), rose bengal (C. I. No. 45435) and a mixture thereof. In general, the content of these colorants is preferably about 1 to 20 parts by weight based on 100 parts by weight of the toner.

The toner according to the present invention can be prepared, for example, by the following method. Specifically, a toner comprising a powder having a desired particle diameter can be prepared by adding a colorant to the mixture of the first polyester and the second polyester and optionally other resin(s), preliminarily mixing them with each other, melt-kneading the mixture and subjecting the kneaded mixture to cooling, granulation, pulverization and classification.

In the present invention, although there is no particular limitation on the particle diameter of the toner, the mean particle size is usually 3 to 30  $\mu\text{m}$ .

If necessary, flow improvers, cleaning improvers, etc. may be incorporated into the toner according to the present invention. Examples of the flow improver include silica, alumina, titanium oxide, barium titanate, magnesium titanate, calcium titanate, strontium titanate, zinc oxide, quartz sand, clay, mica, wollastonite, diatomaceous earth, chromium oxide, cerium oxide, red iron oxide, antimony trioxide, magnesium oxide, zirconium oxide, barium sulfate, barium carbonate, calcium carbonate, silicon carbide and silicon nitride. Impalpable powder of silica is particularly preferred.

The impalpable powder of silica is a fine powder of a compound having a Si-O-Si bond, and may be prepared by either the dry process or the wet process. Although the impalpable powder may contain any of aluminum silicate, sodium silicate, potassium silicate, magnesium silicate and zinc silicate as well as anhydrous silicon dioxide, the impalpable powder containing 85 to 100% by weight of  $\text{SiO}_2$  is preferable. It is also possible to use an impalpable powder of silica subjected to a surface

treatment with a silane coupling agent, a titanium coupling agent, a silicone oil, a silicone oil having an amino group in its side chain and the like in the present invention.

Examples of the cleaning improver include impalpable or fine powders of metal salts of higher fatty acids represented by zinc stearate and fluoropolymers.

Further, it is also possible to use additives for adjusting the developability, for example, an impalpable powder of a polymer of methyl methacrylate.

Further, a minor amount of carbon black may be used for the purpose of adjusting the color tone and resistance. Examples of the carbon black useable in the present invention include various types of carbon black known in the art, for example, furnace black, channel black and acetylene black.

When the toner according to the present invention contains a magnetic impalpable or fine powder, it may be used alone as a developer. On the other hand, when it contains no magnetic impalpable powder, it may be used in the form of a binary developer prepared by mixing it with a carrier. There is no particular limitation on the carrier, and examples thereof include iron powder, ferrite and glass beads or the above-described carriers coated with a resin. The mixing ratio of the toner to the carrier is 0.5 to 10% by weight. The particle diameter of the carrier is 30 to 500  $\mu\text{m}$ . It is also possible to use a nonmagnetic one-component toner without the use of a carrier.

Since the developer composition of the present invention comprises first and second polyesters, each having particular properties, it is excellent in hot offset resistance, low temperature fixation, smoothness and transparency of the fixed face and blocking resistance by virtue of a synergistic effect of these first and second polyesters.

Specifically, the first polyester is a linear polyester and has a relatively high molecular weight. The first polyester, as such, is excellent in hot offset resistance and blocking resistance as well as in the dispersibility of the additives contained therein, so that it can impart excellent transparency to the toner. However, it caused deterioration in the surface smoothness in the low temperature fixation region. On the other hand, the second polyester is a linear polyester having a relatively low molecular weight. As such, it imparts excellent low temperature fixation, smoothness of the fixed face and transparency to the toner. However, it causes deteriora-

tion in the hot offset resistance and blocking resistance. Therefore, when the first polyester and the second polyester are used alone, the respective drawbacks are remarkably exhibited. However, in the developer composition of the present invention, since both the first polyester and the second polyester are present together, the mixture contains the so-called "linearly broadened molecular weight distribution". As a result, to the toner according to the present invention, excellent transparency is imparted by virtue of the presence of the first polyester having a relatively high molecular weight which is excellent in hot offset resistance and blocking resistance as well as in the dispersibility of additives dispersed therein. At the same time, excellent low temperature fixation, smoothness of the fixed face and transparency are imparted by virtue of the presence of the second polyester having a low molecular weight, so that it is possible to attain excellent results whereby low temperature fixation and the smoothness of the fixed face can be significantly improved without adversely affecting the hot offset resistance, blocking resistance and transparency, and furthermore, a toner having excellent properties can be efficiently prepared by the conventional kneading-pulverization process.

## EXAMPLES

The present invention will now be described in more detail with reference to the following Examples which should not be considered to limit the scope of the present invention.

### Production of Polyester

A four neck flask having a capacity of 2 liters and equipped with a thermometer, a stainless steel agitator, a glass nitrogen inlet tube and a falling condenser was charged with components according to the formulation indicated in Table 1 with the further addition of 0.75 g of hydroquinone, and then set in a mantle heater. The contents of the flask were allowed to react with each other at 220°C. and below in a nitrogen atmosphere and under reduced pressure with agitation. The progress of the reaction was monitored by measuring the acid value and the reaction was stopped when the acid value reached a predetermined value. The flask was then cooled to room temperature to produce individual polyesters as a yellow solid form.

The property values of the respective polyesters are given in Table 1.

TABLE 1

| Polyester No. | Monomer for Alcohol Component                                                     |                                                                       |                         | Monomer for Acid component |                     |                           | Properties of resin             |  |
|---------------|-----------------------------------------------------------------------------------|-----------------------------------------------------------------------|-------------------------|----------------------------|---------------------|---------------------------|---------------------------------|--|
|               | polyoxy-<br>polyoxypolypropylene<br>(2.2)-2,2-bis(4-<br>hydroxyphenyl)<br>propane | polyoxy-<br>ethylene(2.0)-<br>2,2-bis(4-<br>hydroxyphenyl)<br>propane | fumaric<br>acid         | succinic<br>acid           | isophthalic<br>acid | softening<br>point<br>Tsp | glass<br>transition<br>point Tg |  |
| 1a            | 1050<br>(3.0 mol)                                                                 | —                                                                     | 348<br>(3.0 mol)        | —                          | —                   | 90°C.                     | 54°C.                           |  |
| 1b            | 1050<br>(3.0 mol)                                                                 | —                                                                     | 348<br>(3.0 mol)        | —                          | —                   | 97                        | 58                              |  |
| 1c            | 1050<br>(3.0 mol)                                                                 | —                                                                     | 348<br>(3.0 mol)        | —                          | —                   | 102                       | 61                              |  |
| 1d            | 1050<br>(3.0 mol)                                                                 | —                                                                     | 348<br>(3.0 mol)        | —                          | —                   | 112                       | 64                              |  |
| 1e            | 1050<br>(3.0 mol)                                                                 | —                                                                     | 348<br>(3.0 mol)        | —                          | —                   | 123                       | 67                              |  |
| 2a            | 1050                                                                              | —                                                                     | —<br>354 g<br>(3.0 mol) | —                          | —                   | 92                        | 53                              |  |
| 2b            | 1050<br>(3.0 mol)                                                                 | —                                                                     | —<br>354 g<br>(3.0 mol) | —                          | —                   | 112                       | 64                              |  |

TABLE 1-continued

| Polyester<br>No. | Monomer for<br>Alcohol Component                              |                                                                   | Monomer for<br>Acid component |                    |                     | Properties of resin                   |                                             |
|------------------|---------------------------------------------------------------|-------------------------------------------------------------------|-------------------------------|--------------------|---------------------|---------------------------------------|---------------------------------------------|
|                  | polyoxypropylene<br>(2.2)-2,2-bis(4-<br>hydroxyphenyl)propane | polyoxy-<br>ethylene(2.0)-<br>2,2-bis(4-<br>hydroxyphenyl)propane | fumaric<br>acid               | succinic<br>acid   | isophthalic<br>acid | softening<br>point<br>T <sub>sp</sub> | glass<br>transition<br>point T <sub>g</sub> |
| 2c               | 1050<br>(3.0 mol)                                             | —                                                                 | —                             | 354 g<br>(3.0 mol) | —                   | 122                                   | 67                                          |
| 3a               | 840<br>(2.4 mol)                                              | 195<br>(0.6 mol)                                                  | 244<br>(2.1 mol)              | —                  | 149<br>(0.9 mol)    | 89                                    | 52                                          |
| 3b               | 840<br>(2.4 mol)                                              | 195<br>(0.6 mol)                                                  | 244<br>(2.1 mol)              | —                  | 149<br>(0.9 mol)    | 113                                   | 63                                          |
| 3c               | 840<br>(2.4 mol)                                              | 195<br>(0.6 mol)                                                  | 244<br>(2.1 mol)              | —                  | 149<br>(0.9 mol)    | 118                                   | 65                                          |

## EXAMPLES 1 TO 6 AND COMPARATIVE EXAMPLES 5 TO 5

In the individual Examples and Comparative Examples, 80 parts by weight in total of the polyesters in combination and blended in the amount indicated in Table 2, 20 parts by weight of styrene-acrylic resin, 1 part by weight of a magenta dye "ROB-B" (manufactured by Orient Chemical Industries, Ltd.), 0.8 part by weight of a charge control agent "Bontron P-51" (manufactured by Orient Chemical Industries, Ltd.) and 2 parts by weight of a low molecular weight polypropylene "Viscol 660P" (softening point, T<sub>sp</sub>, 130° C.; a product of Sanyo Chemical Industries, Ltd.) were preliminarily mixed with each other. Then the resulting mixture was subjected to conventional procedures, i.e., melting, kneading, cooling, grinding and classification, to prepare a particulate powder having a particle diameter of 10  $\mu$ m.

In the step of grinding, the mass, after kneading, was crushed and classified to pass a 9.2 mesh (nominal size: 2 mm)/16 mesh on (nominal size: 1 mm) and finely ground by means of a jet fine grinding mill. 0.3 part by weight of an impalpable powder of hydrophobic silica "Aerosil R-972" was added and mixed with 100 parts by weight of the particulate powder to give a toner according to the present invention.

50 parts by weight of the toner thus obtained was mixed with 950 parts by weight of silicone-coated ferrite carrier (manufactured by Kanto Denka Kogyo Co., Ltd.) by means of a V-shape blender to give a developer.

This developer was used in a two-component dry copying machine equipped with a commercially available organic photoreceptor to obtain an initial image and subjected to a performance evaluation according to the following methods.

## Evaluation Methods

## (1) Minimum Fixation Temperature

An unfixed image was formed within a copying machine, and a test was conducted on a fixation temperature region by means of an external fixing machine. In the fixing roller of the external fixing machine, both upper and lower rollers were coated with a high heat resistant silicone rubber, and a heater was provided within the upper roller.

Toner images formed by the above-described individual toners transferred on a transfer paper having a basis

20 weight of 64 g/m<sup>2</sup> under environmental conditions of a temperature of 20° C. and a relative humidity of 20% were fixed at a linear velocity of 115 mm/sec by means of a heat roller fixing apparatus which was conducted by the stepwise raising of the set temperature of the heat roller from 120° C.

25 In the resultant fixed image, a solid toner having a size of 2 cm × 2 cm was folded in two, and the folded portion was inspected with the naked eye to determine the toner was fixed or not. The minimum preset temperature necessary for obtaining a fixed image was determined. This temperature was viewed as the minimum fixing temperature. The heat roller fixing apparatus is one not equipped with a silicone oil feed mechanism.

## (2) Hot Offset Generation Temperature

According to the above-described measurement of the minimum fixing temperature, a toner image was transferred, a fixation treatment was conducted by means of the above-described heat roller fixing apparatus, and a transfer paper having a white color was fed to the above-described heat roller fixing apparatus under the same conditions to determine with the naked eye whether or not toner staining occurred. The above-described procedure was repeated in such a manner that 40 the preset temperature of the heat roller of the above-described heat roller fixing apparatus was successively raised, thereby determining the minimum preset temperature at which the toner staining occurred. The minimum present temperature was viewed as the hot offset generation temperature.

## (3) Gloss of Fixed Face

At a coverage of 15 mg/cm<sup>2</sup> of the toner on the paper, the gloss of the toner image which formed by fixing 55 at each fixing temperature was measured through the use of a glossmeter "MODEL VG-2PD" manufactured by Nippon Denshoku Co., Ltd..

## (4) Transparency

The transparency of sheet copy for OHP was compared with the color reproducibility of an image projected by OHP. The transparency is measured through the use of SZ-Σ80 manufactured by Nippon Denshoku Co., Ltd.. In this case, the transmittance of a wavelength region of visible light was measured with the transparency of an unused sheet for OHP being supposed to be 100%.

The results are summarized in Table 2.

TABLE 2

| Toner No. | First polyester |                 |             | Second polyester |                 |             | Offset generation temp. | Min. fixation temp. | Gloss   |         |         | Transparency (OHP film) |                       |                    |
|-----------|-----------------|-----------------|-------------|------------------|-----------------|-------------|-------------------------|---------------------|---------|---------|---------|-------------------------|-----------------------|--------------------|
|           | No.             | softening point | amt. of Tsp | No.              | softening point | amt. of Tsp |                         |                     | pts. wt | 160° C. | 180° C. | spectral transmittance  | color reproducibility |                    |
|           |                 |                 |             |                  |                 |             |                         |                     |         |         |         |                         |                       |                    |
| Ex. 1     | toner 1         | 1d              | 112° C.     |                  | 50              |             | 1a                      | 90° C.              | 50      | 200° C. | 150° C. | 8                       | 20                    | 85% bright magenta |
| Ex. 2     | toner 2         | 1e              | 123         |                  | 30              |             | 1a                      | 90                  | 70      | 190     | 160     | 7                       | 18                    | 82 bright magenta  |
| Ex. 3     | toner 3         | 2b              | 112         |                  | 50              |             | 2a                      | 92                  | 50      | 200     | 150     | 7                       | 19                    | 83 bright magenta  |
| Ex. 4     | toner 4         | 2c              | 122         |                  | 30              |             | 2a                      | 92                  | 70      | 200     | 160     | 6                       | 18                    | 81 bright magenta  |
| Ex. 5     | toner 5         | 3b              | 113         |                  | 50              |             | 3a                      | 89                  | 50      | 190     | 150     | 8                       | 16                    | 81 bright magenta  |
| Ex. 6     | toner 6         | 3c              | 118         |                  | 30              |             | 3a                      | 89                  | 70      | 190     | 150     | 7                       | 15                    | 80 bright magenta  |
| Comp.     | comp.           | 1b              | 97° C.      |                  | 50              |             | 1a                      | 90                  | 50      | 160     | 150     | —                       | —                     | —                  |
| Ex. 1     | toner 1         |                 |             |                  | pts. wt         |             | 1d                      | 112                 | 70      | 210     | 170     | —                       | 6                     | 72 dark magenta    |
| Comp.     | comp.           | 1e              | 123         |                  | 30              |             |                         |                     |         |         |         |                         |                       | dark magenta       |
| Ex. 2     | toner 2         |                 |             |                  |                 |             |                         |                     |         |         |         |                         |                       | dark magenta       |
| Comp.     | comp.           | 1d              | 112         |                  | 100             |             | —                       | —                   | —       | 210     | 170     | —                       | 7                     | 74                 |
| Ex. 3     | toner 3         |                 |             |                  |                 |             |                         |                     |         |         |         |                         |                       | —                  |
| Comp.     | comp.           | —               | —           |                  | —               |             | 2a                      | 92                  | 100     | 150     | 140     | —                       | —                     | —                  |
| Ex. 4     | toner 4         |                 |             |                  |                 |             |                         |                     |         |         |         |                         |                       | —                  |
| Comp.     | comp.           | 1c              | 102         |                  | 50              |             | 1b                      | 97                  | 50      | 170     | 150     | 15                      | —                     | —                  |
| Ex. 5     | toner 5         |                 |             |                  |                 |             |                         |                     |         |         |         |                         |                       | —                  |

Further, the above-described toners 1 to 6 were allowed to stand under environmental conditions at a temperature of 45° C. and a relative humidity of 26% for 2 weeks, and the blocking resistance was evaluated based on whether or not agglomeration occurs in each toner. As a result, no agglomerate was observed, and the blocking resistance was excellent.

As can be understood from the above-described results, all the toners 1 to 6 of the present invention were excellent in hot offset resistance, low temperature fixation, gloss of fixed face, transparency and blocking resistance, and it is possible to prepare a toner which is excellent particularly in its heat characteristics.

By contrast, the comparative toner 1 is poor in hot offset resistance because the softening point, Tsp, of the first polyester is below 105° C.

The comparative toner 2 is poor in low temperature fixation, gloss of fixed surface and transparency because the softening point, Tsp, of the second polyester is not below 105° C.

The comparative toner 3 is poor in low temperature fixation, gloss and transparency because it contains no second polyester.

The comparative toner 4 is poor in hot offset resistance because it contains no first polyester.

The comparative toner 5 is poor in hot offset resistance because the difference in the softening point, Tsp, between the first polyester and the second polyester is less than 10° C.

The invention being thus described, it will be obvious that the same may be varied in many ways. Such variations are not to be regarded as a departure from the spirit and scope of the invention, and all such modifications as would be obvious to one skilled in the art are intended to be included within the scope of the following claims.

What we claim:

1. A developer composition for electrophotography comprising a binding resin and a colorant, said binding resin comprising a first linear polyester having a softening point, Tsp, in the range of from 105° C. to 170° C. exclusive, and a second linear polyester having a softening point, Tsp, in the range of from 80° C. to 105° C.

30 exclusive and lower than that of the first linear polyester by at least 10° C., the weight ratio of the first linear polyester to the second linear polyester being (80:20) to (20:80).

2. The developer composition for electrophotography according to claim 1, wherein the first linear polyester and the second linear polyester each comprises an acid component originated from an aliphatic dicarboxylic acid and/or acid anhydride thereof in an amount of 50% and more by mole based on the entire acid component.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070

and 30 to 0% by weight of styrene-acrylic resin based on the entire binding resin.

7. The developer composition for electrophotography according to claim 1, wherein the developer com-

position further comprises a low molecular weight polyolefin.

8. The developer composition for electrophotography according to claim 1, wherein the developer composition further comprises a magnetic impalpable powder.

\* \* \* \* \*

10

15

20

25

30

35

40

45

50

55

60

65